

Patented Nov. 13, 1928.

1,691,661

# UNITED STATES PATENT OFFICE.

IRVING F. LAUCKS AND GLENN DAVIDSON, OF SEATTLE, WASHINGTON, ASSIGNEES TO  
I. F. LAUCKS, INC., OF SEATTLE, WASHINGTON, A CORPORATION OF WASHINGTON.

## VEGETABLE GLUE AND METHOD OF MAKING SAME.

No Drawing. Original application filed October 29, 1923, Serial No. 671,381. Divided and this application filed March 9, 1927. Serial No. 174,093.

The art of making a water-proof glue from certain protein materials has been known for some time; thus casein and blood albumin are in common use. These last mentioned 5 compounds, however, have a number of disadvantages from a practical standpoint. Casein is costly and lack of uniformity in the material as derived from various sources is a serious detriment; while blood albumin is 10 not available except in certain situations. There is accordingly a great demand, particularly in the veneer industry where large quantities of glue are consumed, for a new glue that will be cheap and at the same time 15 sufficiently water-proof.

By water-proof, in this connection, it is not meant that glues thus characterized will resist the action of water indefinitely, but it is meant that they are water-proof in the 20 sense in which the term is used in the veneer industry, viz., that a panel can be soaked in cold water for from seventy-two to one hundred hours, or in boiling water for eight hours, without separation.

25 Vegetable compounds have not, so far as we are aware, been heretofore satisfactorily employed as a basis for water-proof glues of the type in question. It is true that some veneer makers, on account of the high price 30 of casein, have come to use starch glues but these, at least as heretofore made, are not at all water-proof, and vegetable proteins have not heretofore been used at all, so far as we are aware.

35 We have now discovered, however, that by subjecting the same to proper treatment, such vegetable proteins or vegetable matter containing proteins in proper amount can be converted into a water-proof glue that will satisfy the rigid requirements of veneer making. The requisite raw material may be derived 40 from a number of sources and the treatment of such material according to our invention is relatively simple and inexpensive so that 45 as a result we are able to produce a satisfactory glue at a much lower cost than has heretofore been possible.

To the accomplishment of the foregoing and related ends, the invention, then, consists 50 of the combination of ingredients or composition of matter and the steps involved in the preparation of such composition hereinafter fully described and particularly pointed out

in the claims, it being understood that such disclosed ingredients and steps constitute but 55 several of the various ways in which the principle of the invention may be used.

We have found that soya bean flour constitutes an admirable raw material for our 60 purpose. Such flour is preferably made by grinding soya bean cake so that 80 per cent will pass a 100 mesh screen and when treated with certain chemicals, or other substances, we make therefrom a very satisfactory glue 65 that meets the requirements of the veneer trade fully and is in many respects better than the usual glues now on the market. Such bean cake, as analyzed by us, is found to contain on the average 45 per cent protein, 12 70 per cent water, 5 per cent cellulose or crude fiber, 7 per cent oil, 6 per cent ash, and 25 per cent carbohydrates.

We do not, however, wish to limit ourselves 75 to soya bean flour or to vegetable protein derived from this source for we have made satisfactory glue by our improved process from a low grade wheat containing approximately 10 per cent protein and there are many other 80 vegetable materials containing protein in amounts intermediate between the percentages thus noted as found in such soya bean flour and wheat or even lower than the percentage in such wheat that may be utilized with satisfactory results; that is, soya bean flour gives the best results, but other sources 85 of vegetable protein-containing material may be employed with proportionately advantageous results.

Soya bean flour made from soya bean cake 90 from which the oil has been expressed, is preferably used in practice because it is cheaper and makes a better glue, but flour made from whole soya beans, without expressing the contained oil, may also be used, 95 although obviously this would not be economical in view of the value which attaches to such oil. As to the fineness of the flour, it is not necessary that the meal be ground as fine as indicated above, but fineness is desirable from a practical standpoint.

When the usual chemicals employed in 100 making casein glue, viz., lime and sodium silicate, are added to a vegetable protein-containing material, for example, soya bean flour, a glue results, but it is not as good as casein glue. It is not as highly water resist-

- ant nor as workable. We find, however, by the use of caustic soda with such vegetable protein-containing matter, a much better glue is obtained, such caustic soda apparently 5 playing the part of dispersing the colloidal material. The resultant glue is then somewhat similar in its working properties to casein glue, although its water resistance is still slightly less.
- 10 Desirably we employ an agent which responds to the following test, viz, if said agent is placed in dilute water solution, it furnishes hydroxyl ions. Compounds responding to this test are commonly called alkaline com- 15 pounds and in water solution would provide an alkaline medium. Preferably we react on our vegetable protein-containing material with both caustic soda and lime. As equivalents of such caustic soda, caustic potash 20 and ammonia may be used, although more expensive. Other equivalents of caustic soda are salts of soda (or potash) with weak acids, e. g. sodium phosphate, sodium borate and the like. Similarly in place of lime, magnesia, baryta and strontia may be used as equivalents.

In order to improve the working properties, e. g. the spreading and flow, of the glue produced as aforesaid as well as the water 30 resisting properties, we have found it desirable to add other substances of which the following are examples:—

Carbon bisulphide, calcium polysulphide. Equivalents would be other sulphur com- 35 pounds of like properties or constitution, such as, for example, sodium thiocarbonate and potassium xanthate, sodium silicate, or other soluble silicates.

In general carbon-bisulphide imparts very 40 great water resisting properties, as does also calcium polysulphide, although to a lesser degree, that is, for good practical effects sulphur-containing compounds like carbon bisulphide which in the composition with the 45 vegetable protein matter provide sulphur derivatives of carbonic acid are most desirably employed,—such sulphur derivatives of carbonic acid constituting a regularly recognized classification in standard chemical authorities, such, for example, as Richter, Organic 50 Chemistry, 1916, Volume I, page 431, and Julius Schmidt, Organic Chemistry, page 298.

In connection with this general treatment, 55 we also bring the vegetable protein-containing matter into a dispersed condition; that is, the state attained in the transformation of a mealy-like or granular mass to a more or less smooth mass in the presence of a liquid, and to such extent as we thus refer to the degree of subdivision of particles we believe that we are using the term dispersion not inconsistently with the accepted usage of colloid chemists.

60 We have also found that certain substances

will act in the same way as the caustic soda and also render the product of a very desirable consistency, e. g. sodium phosphate, sodium perborate and sodium sulphite. These salts are all related in that they are combinations of the strong base sodium with a weak acid and there are a number of other salts that fall in the same category and which have a similar effect, so need not be listed in detail.

75 As examples we may cite the following typical formulæ:—

1. Mix 30 parts soya bean flour with 120 parts water; add 13 parts of 18 per cent caustic soda solution and mix; 5 parts carbon bisulphide are then added and stirred well; to this 3 parts calcium hydrate are added and stirred in; then 15 parts water glass (sodium silicate) are stirred in; finally, add 1 part copper sulphate to 5 parts of water and stir in. This makes the finished glue, which is then spread on panels, for example, put under pressure for several hours, whereupon the pressure may be released.

80 2. Dry mix 900 parts peanut flour; 90 parts sodium carbonate; 54 parts lime; and 67½ parts sodium fluoride; this dry mixture is added to 1800 parts of water with stirring and then is added 18 parts lime suspended in 15 parts of water and 30 parts of carbon bisulphide; this mixture is again stirred and then to the same is added 2000 parts of water and the stirring continued for about ten minutes which provides the finished adhesive or glue.

90 3. The dry mixture is the same here as in Example No. 2 excepting cottonseed flour is substituted for peanut flour; to the dry mixture 1500 parts of water are added and 15 parts lime in 15 parts of water and 90 parts 95 of sodium thiocarbonate solution; to this mixture is added 1900 parts of water, stirring the same as in Example 2; the sodium thiocarbonate solution is prepared by dissolving 320 parts of 60 per cent sodium sulphide 100 in 1000 parts of water and adding 260 parts of carbon bisulphide.

105 4. Dry mix 300 parts of soya bean flour; 65 parts of lime; 30 parts of sodium carbonate; 22½ parts of sodium fluoride; and 10 110 parts of boric acid; to this dry mixture is then added 650 parts of water with stirring; then 25 parts of potassium xanthate is added with stirring; next is added 400 parts of water with stirring which stirring is continued for about ten minutes.

115 The particular order in which the several ingredients are admixed together in the formulæ just given may be varied and it is not necessary that the manufacture of the product 120 be completed in a single continuous operation, but as a matter of practice we have found it desirable in certain cases to mix only certain 125 of the ingredients initially and then add the others just before the glue is required for use,

75  
80  
85  
90  
95  
100

90  
95  
100

105  
110  
115

120  
125  
130

that is, the dry ingredients or, as the same may be called, the dry mix of the above examples may be supplied to the user unassociated with the liquid ingredients and the liquid ingredients then added by the user at the time he wishes to prepare the adhesive.

It will also be understood, of course, that the foregoing formulæ are typical and that many variations are actually made therein 10 in the compounding of our improved glue.

This application is a division of our application, Serial No. 671,381, filed Oct. 29, 1923.

Other modes of applying the principle of 15 our invention may be employed instead of the one explained, change being made as regards the process herein disclosed or the materials employed in carrying out such process provided the stated ingredients and steps or the 20 equivalent of such stated ingredients or steps be employed.

We therefore particularly point out and distinctly claim as our invention:—

1. An adhesive which comprises the reaction products of vegetable protein matter, an aqueous alkaline medium, and a small proportion of a sulphur-containing compound which provides a sulphur derivative of carbonic acid.

30 2. An adhesive which comprises the reaction products of vegetable protein matter, an aqueous caustic soda medium, and a small proportion of a sulphur-containing compound which provides a sulphur derivative 35 of carbonic acid.

3. An adhesive which comprises the reaction products of vegetable protein matter, an aqueous caustic soda-lime medium, and a small proportion of a sulphur-containing compound which provides a sulphur derivative 40 of carbonic acid.

4. An adhesive which comprises the reaction products of soya bean protein matter, an aqueous alkaline medium, and a small proportion of a sulphur-containing compound which provides a sulphur derivative of carbonic acid.

5. An adhesive which comprises the reaction products of soya bean protein matter, an aqueous caustic soda medium, and a small proportion of a sulphur-containing compound which provides a sulphur derivative of carbonic acid.

6. An adhesive which comprises the reaction products of soya bean protein matter, an aqueous caustic soda-lime medium, and a small proportion of a sulphur-containing compound which provides a sulphur derivative of carbonic acid.

60 7. An adhesive which comprises the reaction products of vegetable protein matter, an aqueous alkaline medium, and a small proportion of carbon bisulphide.

8. An adhesive which comprises the reaction products of vegetable protein matter,

an aqueous caustic soda medium, and a small proportion of carbon bisulphide.

9. An adhesive which comprises the reaction products of vegetable protein matter, an aqueous caustic soda-lime medium, and a small proportion of carbon bisulphide.

10. An adhesive which comprises the reaction products of soya bean protein matter, an aqueous alkaline medium, and a small proportion of carbon bisulphide.

11. An adhesive which comprises the reaction products of soya bean protein matter, an aqueous caustic soda medium, and a small proportion of carbon bisulphide.

12. An adhesive which comprises the reaction products of soya bean protein matter, an aqueous caustic soda-lime medium, and a small proportion of carbon bisulphide.

13. An adhesive which comprises the reaction products of soya bean flour, an aqueous alkaline medium, and carbon bisulphide as a water-proofing agent.

14. An adhesive which comprises the reaction products of soya bean flour, an aqueous alkaline medium, and carbon bisulphide, the carbon bisulphide and the soya bean flour being in the proportions of about five parts and about thirty parts respectively.

15. In an aqueous vegetable protein-containing adhesive an ingredient which functions as a water-resistance-increasing agent, the same being the reaction product of a sulphur-containing compound which provides a sulphur derivative of carbonic acid.

16. In an aqueous vegetable protein-containing adhesive an ingredient which functions as a water-resistance-increasing agent, the same being the reaction product of carbon bisulphide therewith.

17. In an aqueous soya bean protein-containing adhesive an ingredient which functions as a water-resistance-increasing agent, the same being the reaction product of a sulphur-containing compound which provides a sulphur derivative of carbonic acid.

18. In an aqueous soya bean protein-containing adhesive an ingredient which functions as a water-resistance-increasing agent, the same being the reaction product of carbon bisulphide therewith.

19. In the process of making an adhesive, the step of reacting upon alkaline treated vegetable protein matter in an aqueous medium with a small proportion of a sulphur-containing compound which provides a sulphur derivative of carbonic acid.

20. In the process of making an adhesive, the step of reacting upon alkaline treated vegetable protein matter in an aqueous medium with a small proportion of carbon bisulphide.

21. In the process of making an adhesive, the step of reacting upon alkaline treated soya bean protein matter in an aqueous medium with a small proportion of a sulphur-

- containing compound which provides a sulphur derivative of carbonic acid.
22. In the process of making an adhesive, the step of reacting upon alkaline treated soya bean protein matter in an aqueous medium with a small proportion of carbon bisulphide.
23. The process of making an adhesive, comprising subjecting vegetable protein matter to an aqueous alkaline medium of a strength which will chemically react with such protein matter in the presence of a small proportion of a sulphur-containing compound which provides a sulphur derivative of carbonic acid.
24. The process of making an adhesive, comprising reacting upon vegetable protein matter in an aqueous caustic soda medium with a small proportion of sulphur-containing compound which provides a sulphur derivative of carbonic acid.
25. The process of making an adhesive, comprising reacting upon vegetable protein matter in an aqueous caustic soda-lime medium with a small proportion of a sulphur containing compound which provides a sulphur derivative of carbonic acid.
26. The process of making an adhesive, comprising subjecting soya bean protein matter to an aqueous alkaline medium of a strength which will chemically react with such protein matter in the presence of a small proportion of a sulphur-containing compound which provides a sulphur derivative of carbonic acid.
27. The process of making an adhesive, comprising reacting upon soya bean protein matter in an aqueous caustic soda medium with a small proportion of a sulphur-containing compound which provides a sulphur derivative of carbonic acid.
28. The process of making an adhesive, comprising reacting upon soya bean protein matter in an aqueous caustic soda-lime medium with a small proportion of a sulphur-containing compound which provides a sulphur derivative of carbonic acid.
29. The process of making an adhesive, comprising subjecting vegetable protein matter to an aqueous alkaline medium of a strength which will chemically react with such protein matter in the presence of a small proportion of carbon bisulphide.
30. The process of making an adhesive, comprising reacting upon vegetable protein matter in an aqueous caustic soda medium with a small proportion of carbon bisulphide.
31. The process of making an adhesive, comprising reacting upon vegetable protein matter in an aqueous caustic soda-lime me-
- dium with a small proportion of carbon bisulphide.
32. The process of making an adhesive comprising subjecting soya bean protein matter to an aqueous alkaline medium of a strength which will chemically react with such protein matter in the presence of a small proportion of carbon bisulphide.
33. The process of making an adhesive, comprising reacting upon soya bean protein matter in an aqueous caustic soda medium with a small proportion of carbon bisulphide.
34. The process of making an adhesive, comprising reacting upon soya bean protein matter in an aqueous caustic soda-lime medium with a small proportion of carbon bisulphide.
35. The process of making an adhesive, comprising subjecting vegetable protein matter to an aqueous alkaline medium of a strength which will chemically react with such protein matter in the presence of a small proportion of a liquid sulphur-containing compound which provides a sulphur derivative of carbonic acid.
36. The process of making an adhesive, comprising reacting upon vegetable protein matter in an aqueous caustic soda medium with a small proportion of a liquid sulphur containing compound which provides a sulphur derivative of carbonic acid.
37. The process of making an adhesive, comprising reacting upon vegetable protein matter in an aqueous caustic soda-lime medium with a small proportion of a liquid sulphur-containing compound which provides a sulphur derivative of carbonic acid.
38. The process of making an adhesive, comprising subjecting soya bean protein matter to an aqueous alkaline medium of a strength which will chemically react with such protein matter in the presence of a small proportion of a liquid sulphur containing compound which provides a sulphur derivative of carbonic acid.
39. The process of making an adhesive, comprising reacting upon soya bean protein matter in an aqueous caustic soda medium with a small proportion of a liquid sulphur-containing compound which provides a sulphur derivative of carbonic acid.
40. The process of making an adhesive, comprising reacting upon soya bean protein matter in an aqueous caustic soda-lime medium with a small proportion of a liquid sulphur-containing compound which provides a sulphur derivative of carbonic acid.

Signed by us this first day of March, 1927.

IRVING F. LAUCKS.  
GLENN DAVIDSON.